# EUROPEAN PATENT SPECIFICATION

(11) **EP 0 148 539 B1**
(45) Date of publication and mention of the grant of the patent: **25.11.1987**
(21) Application number: 84300092.8
(22) Date of filing: 06.01.1984
(51) Int. Cl.: D04H 1/46

(54) **Process for producing a ceramic fiber blanket**
Verfahren zur Herstellung einer Keramikfasermatte
Procédé de fabrication d'un mât de fibres de céramique

(43) Date of publication of application: 17.07.1985
(73) Proprietor: ISOLITE BABCOCK REFRACTORIES COMPANY LIMITED, Hoi-Gun, Aichi-Ken (JP)
(72) Inventor: Yamanaka, Hideki, Toyokawa City Aichi Prefecture (JP)
(74) Representative: Hartley, David

## Description

The present invention relates to a process for producing a ceramic fibre blanket.

Japanese Patent specification No. 153/65 discloses a process for producing a ceramic fibre blanket comprising alumina and silica, in which a fine falling stream of molten kaolin or like material is converted into staple fibres by blowing, spinning or other suitable method, the filaments are blended with a lubricant, and a web of the blend is placed on a belt conveyor and pressed between wire screens as it is heated to evaporate the lubricant. In a web of fibres that has been simply compressed without blending the fibres with a lubricant, the individual fibres are not interlinked and disintegrate easily, so the web provides only a laminar structure of a very low strength that is difficult to handle. But if a web of fibres treated with a lubricant is compressed as it is heated to remove the lubricant, the fibres remain interlinked after the compression and provide a laminar structure that has strength high enough to withstand subsequent handling.

When a ceramic fibre blanket not more than about 5 mm thick is produced by this conventional method, a meshed or roller conveyor is used to facilitate evaporation of the lubricant during compression, with the result that the mesh pattern is impressed on both surfaces of the blanket and the recessed part is so thin as to be transparent, while in case of the roller conveyor there provides an error in the dimension of the blanket, as the process is carried out in the heated condition. To eliminate this problem and provide a uniformly thin blanket, short fibres capable of being uniformly dispersed in water are dispersed in water in the presence of a binder and a sheet of ceramic fibre is produced by the conventional paper-making method. This wet process however, needs much labour and has low fibre utility due to loss of fibre dust that accompanies the fibre cutting step.

One object of the present invention is to facilitate the manufacture of a ceramic fibre blanket having adequate strength.

In accordance with the present invention we propose a process for producing a ceramic fibre blanket comprising the steps of preparing a laminar pile of ceramic fibres superimposing a web of organic fibres on one or both sides of the pile, and punching the resulting assembly with barbed needles, characterised in that the laminar pile of ceramic fibre comprises 35 to 65% by weight of alumina, 35 to 65% by weight of silica, less than 10% by weight of another metal oxide and a lubricant, the lubricant being removed after punching by incineration without application of pressure.

Japanese Patent Publication No. 43946/77 describes a process for making a ceramic fibre blanket wherein a web of ceramic fibres treated with a lubricant is punched with barbed needles and then the lubricant is removed under pressure. This produces a product having a greater tensile strength than the blanket made by removing the lubricant under pressure without needle punching. But even this method does not provide a uniformly thin blanket since the meshed or roller conveyor such as referred to above is used to compress the web during elimination of the lubricant.

Furthermore, if more than 40 needles are punched through an area of one square centimeter in an attempt to provide a greater tensile strength, the web stretches in four directions and tends to rupture. A thin web is inherently weaker than a thick one and increasing the punching density to provide the thin pile with the same tensile strength as that of the thick one only results in a ruptured blanket.

Japanese Patent application (OPI) No. 77665/75 (the symbol OPI here used means an unexamined published Japanese Patent application) and FR-A-2 248 937 both describe a method of punching barbed needles through a mat of inorganic nonwoven fibres that is free from a lubricant and on which a web of organic nonwoven fibres is superimposed. The needled fibres from the web extend into the mat of nonwoven inorganic fibres to hold the mat and the web together and the mat of the inorganic fibres will return to its initial bulk density by itself after the organic fibres are eliminated (by being burned off prior to or during use). The inorganic fibres do not become interlinked with each other.

It has now been found that if a web of organic fibres is superimposed on one or both surface of a web of ceramic fibres containing a lubricant, more needles/unit area (than in the method of Japanese Patent publication No. 43946/77) can be used without rupturing the web. Further, we have found that if the lubricant is removed from the punched web without application of pressure and if the web of organic fibres is subsequently removed, a blanket or felt that retains the interlinking between the individual ceramic fibres provided by the needle punching is produced.

If only a web of ceramic fibres containing a lubricant is punched with more than 40 needles per square centimeter, the web ruptures, but in the process of the present invention, rupturing will not occur even if the punching density is greater than 40 needles/cm^{2.} This is probably because the organic fibres drawn into the ceramic fibre web with the needles absorb the impact of the needles and prevent separation of the ceramic fibres.

If a lubricant is removed from the punched ceramic fibre web in the absence of pressure and if the web of organic fibres is then removed by incineration, the bulk density of the web will not return to the initial value before the punching and the resulting product retains the effect of the punching and has a great tensile strength. This is probably because the lubricant is removed from the ceramic fibre web that are sewn tightly with the organic fibres and pressure is not necessary to retain the punching effect given the ceramic fibres.

Fats and oils are generally used as the lubricant. They are evaporated from the pile of ceramic fibre web by heating before the organic fibres are incinerated, and throughout the evaporation of the lubricant, the organic fibres retain their effect to clamp the ceramic fibres.

The web of organic fibres is generally made by a carding staple fibres usually of 1.5 to 5 deniers, and 30 to 100 mm long. It can have a density of 30 g/m² or more. The carded web can be immediately used in the present invention, but for ease of handling, the web is preferably punched by barbed needles, and a web having a density of 30 g/m² can be used with satisfactory results. A ceramic fibre blanket having a satisfactory tensile strength and a uniform thickness of 5 mm or less can be produced by punching the above characterised ceramic fibre web with 50 to 200 needles per square centimeter that could not be used in the conventional technique without rupturing the pile. Needless to say, the present invention can also be used to make thicker ceramic fibre blankets.

Embodiments of the present invention will now be described with reference to the following examples.

### Example

A composition of 48 wt% alumina, 52 wt% silica and a trace amount of impurities was melted in an electric furnace and converted into staple fibres by blowing. The ceramic fibres were sprayed with a lubricant which was a 0.5 wt% aqueous emulsion of a 1:5 (by volume) of aliphatic acid amine acetate (Armac HT^{R}) and kerosene, and they were then piled on a belt conveyor to form a web of ceramic fibres. The web had a density of about 530 g/m² (without the lubricant), an average fibre diameter of 2.8 pm and a maximum fibre length of about 250 mm.

Polyester fibres having a fineness of 3 deniers and a length of 76 mm were carded into a web which was punched with 80 needles per square centimeter to give a density of 50 g/m². The punched web was unrolled and superimposed on either the top surface or both surfaces of the ceramic fibre web, and the assembly was punched through both from above and from below with the number of needles varied as indicated in Table 1. The punched assembly was heated in an oven at 500°C for 30 minutes in the absence of pressure to thereby remove the lubricant and polyester fibres successively. Five ceramic fibre blankets (or sheets) were produced by the above procedure, and the bulk density, weight per unit area and tensile strength of each blanket are listed in Table 1.

A ceramic fibre blanket was prepared by the method described in Japanese Patent publication No. 43946/77, wherein a web of ceramic fibres containing a lubricant was punched without laying thereon a web of organic fibres and was then heated under pressure to remove the lubricant. A maximum tensile strength was obtained when the punching density was about 20 needles per square centimeter, but a product having a bulk density of 0.13 and a thickness of 6 mm had a tensile strength of only 0.35 kg/cm² and a product having a bulk density of 0.16 and a thickness of 20.2 mm had a densile strength of 0.9 kg/cm².

When the web of ceramic fibres used in each sample was punched after treatment with the lubricant but without laying up an organic fibre web, the ceramic fibre web ruptured at a punching density of 40 needles/cm².

The present invention makes it possible to manufacture a ceramic fibre blanket having a greater tensile strength that has been unobtainable by conventional techniques, and what is more, a thin blanket that can only be produced by the conventional paper-making method can also be obtained. As shown in the Example, the punching density should not exceed 200 needles per square centimeter when the finished product is to be thinner than about 4 mm, since otherwise the tensile strength of the product is less than that obtained using 150 needles/cm² and the ceramic fibres in the blanket begin to deteriorate. If necessary, the web of organic fibres to be laid up on the ceramic fibre pipe may be treated with a lubricant.

The blanket produced in accordance with the present invention is usually incinerated as in the Example to remove the organic fibres and used as a product containing only ceramic fibres. If necessary, only the lubricant may be removed to provide a blanket with a web of organic fibres which may be removed by incineration attendant to the blanket service.

## Claims

1. A process for producing a ceramic fibre blanket comprising the steps of preparing a laminar pile of ceramic fibres superimposing a web of organic fibres on one or both sides of the pile, and punching the resulting assembly with barbed needles characterised in that the laminar pile of ceramic fibres comprises 35 to 65% by weight of alumina, 35 to 65% by weight of silica, less than 10% by weight of another metal oxide and a lubricant, the lubricant being removed after punching by incineration without application of pressure.

2. A process according to claim 1 wherein the organic fibres are also removed by incineration.

3. A process according to claim 1 wherein the assembly is punched with 50 to 200 barbed needles per square centimeter.

## Patentansprüche

1. Verfahren zur Herstellung einer Keramikfasermatte, indem eine laminare Schicht aus Keramikfasern hergestellt wird, diese Schicht auf einer oder beiden Seiten mit einem Gewerbe aus organischen Fasern überlagert und das entstandene Gebilde mittels mit Widerhaken versehenen Nadeln vernadelt wird, dadurch gekennzeichnet, daß die laminare Schicht aus Keramikfasern 35 bis 65 Gewichtsprozent Aluminiumoxid, 35 bis 65 Gewichtsprozent Kieselsäure, weniger als 10 Gewichtsprozent eines weiteren Metalloxids sowie ein Gleitmittel enthält, wobei das Gleitmittel nach dem Vernadeln durch Veraschung ohne Anwendung von Druck beseitigt wird.

2. Verfahren nach Anspruch 1, dadurch gekennzeichnet, daß auch die organischen Fasern durch Veraschung beseitigt werden.

3. Verfahren nach Anspruch 1, dadurch gekennzeichnet, daß das Gebilde je cm² mittels 50 bis 200 mit Widerhaken versehenen Nadeln vernadelt wird.

## Revendications

1. Procédé de fabrication d'un matelas de fibres de céramique comportant les étapes de préparation d'un empilage laminaire de fibres de céramique en plaçant un voile de fibres organiques sur l'une ou sur les deux faces de l'empilage et d'aiguilletage de l'assemblage obtenu avec des aiguilles à barbes, caractérisé en ce que l'empilage laminaire de fibres de céramique renferme de 35 à 65% en poids d'alumine, de 35 à 65% en poids de silice, moins de 10% en poids d'un autre oxyde métallique et un lubrifiant, le lubrifiant étant éliminé après aiguilletage par incinération sans application de pression.

2. Procédé selon la revendication 1 dans lequel les fibres organiques sont aussi éliminées par incinération.

3. Procédé selon la revendication 1 dans lequel l'assemblage est aiguilleté à l'aide de 50 à 200 aiguilles à barbes par centimère carré.
